

# United States Patent

Takamizawa et al.

[15] 3,639,247

[45] Feb. 1, 1972

[54] **CALCIUM-VANADIUM SERIES  
FERRIMAGNETIC GARNETS**

[72] Inventors: **Hideo Takamizawa; Keiichi Yotsuyanagi; Takashi Okada**, all of Tokyo, Japan

[73] Assignee: **Nippon Electric Company Limited**, Tokyo, Japan

[22] Filed: **Feb. 4, 1970**

[21] Appl. No.: **8,491**

[30] **Foreign Application Priority Data**

Feb. 7, 1969 Japan.....44/9410  
June 27, 1969 Japan.....44/51190

[52] U.S. Cl.....252/62.57,  
252/62.56, 252/62.59, 252/62.63

[51] Int. Cl.....C04b 35/26, C04b 35/40

[58] Field of Search .....252/62.56, 62.57, 62.59, 62.63

[56] **References Cited**

UNITED STATES PATENTS

3,156,651 11/1964 Geller .....252/62.59 X

3,268,452 8/1966 Geller .....252/62.57 X  
3,281,363 10/1966 Geller et al. .....252/62.59 X  
3,291,740 12/1966 Espinosa et al. .....252/62.57 X

Primary Examiner—Tobias E. Levow

Assistant Examiner—J. Cooper

Attorney—Sandoe, Hopgood and Calimafde

[57] **ABSTRACT**

Calcium-vanadium ferrimagnetic garnets having the compositions expressed by the formula:

$\{Ca_{3-y}Y_y\}[Fe_2](Fe_{1.5-0.5x+0.5y}Ge_xV_{1.5-0.5x-0.5y})O_{12}$ ,  
wherein values of  $x$  and  $y$  lie within the polygonal area  
A-B-C-D-E shown in FIG. 7 of the drawing which is  
bounded by the lines connecting the coordinates:

|   | <b>x</b> | <b>y</b> |
|---|----------|----------|
| A | 0.05     | 0.05     |
| B | 0.8      | 0.05     |
| C | 1.8      | 1.1      |
| D | 0.5      | 2.4      |
| E | 0.05     | 2.4      |

and wherein the range expressed by the relation  
 $0.95 \leq y - z \leq 1.05$  is excluded from said area.

**3 Claims, 13 Drawing Figures**

SHEET 1 OF 6



FIG. 1



FIG. 2

INVENTORS  
HIDEO TAKAMIZAWA  
KEIICHI YOTSUYANAGI  
TAKASHI OKADA  
BY

Sandoe, Hopgood & Calmanoff  
ATTORNEYS



FIG. 3



FIG. 4

INVENTORS  
 HIDEO TAKAMIZAWA  
 KEIICHI YOTSUYANAGI  
 TAKASHI OKADA

Sendel, Hopgood & Calimafde  
 ATTORNEYS

PATENTED FEB 1 1972

3,639,247

SHEET 3 OF 6



FIG.5



FIG.6

INVENTORS  
HIDEO TAKAMIZAWA  
KEIICHI YOTSUYANAGI  
BY TAKASHI OKADA

Sandoe, Hopgood & Celmaffle  
ATTORNEYS

PATENTED FEB 1 1972

3 639,247

SHEET 4 OF 6



FIG. 7



FIG. 8

INVENTORS  
HIDEO TAKAMIZAWA  
KEIICHI YOTSUYANAGI  
TAKASHI OKADA  
BY

Sandoe, Hopgood & Calhoun  
ATTORNEYS

PATENTED FEB 1 1972

3,639,247

SHEET 5 OF 6



FIG. 11



FIG. 10

INVENTORS  
HIDEO TAKAMIZAWA  
KEIICHI YOTSUYANAGI  
TAMASHI OKADA  
BY

Sandoe, Hopgood & Calhoun  
ATTORNEYS

PATENTED FEB 1 1972

3,639,247

SHEET 6 OF 6



FIG. 12



FIG. 13

INVENTORS  
HIDEO TAKAMIZAWA  
KEIICHI YOTSUYANAGI  
TAKASHI OKADA  
BY

Sandoe, Hopgood & Calimafde  
ATTORNEYS

## CALCIUM-VANADIUM SERIES FERRIMAGNETIC GARNETS

The present invention relates to calcium-vanadium (Ca-V) series ferrimagnetic garnets for use in microwave circuit elements operating in the VHF, UHF or SHF band range. Among the required characteristics of magnetic materials for use in such microwave circuit elements are low magnetic losses and small temperature variations of the saturation magnetization values ( $4\pi Ms$ ). Desired values of  $4\pi Ms$  will vary according to the application of the magnetic materials. The essential condition for reducing the magnetic loss is that the ferromagnetic resonance linewidth ( $\Delta H$ ) be as low as possible. It has been known that the higher the Curie temperature, the lower becomes the temperature variation of the saturation magnetization ( $4\pi Ms$ ) and that in order to lower the value of the linewidth ( $\Delta H$ ), which is subject to change with the sintering density and the presence or absence of a second phase, the sintering densities must be made sufficiently large and there should be no second phase formation. The yttrium-iron series garnets (YIG) that have been most commonly used as magnetic materials in microwave applications offer the advantages of lower  $4\pi Ms$  values, higher Curie temperatures and lower magnetic losses than conventional spinel-type ferrites such as nickel series ferrites or magnesium-manganese series ferrites. These advantages of the yttrium-iron series garnets are considerably offset by defects such as the necessity for the use of yttrium oxide which is an expensive raw material and the need for sintering at extremely high temperatures and for long time intervals which are not suited for large-scale industrial production. Yttrium-iron garnets substituted with  $Al_2O_3$  for lowering the saturation magnetization have an other defect of a rapid lowering of the Curie temperature which inevitably causes a large variation of  $4\pi Ms$  with a temperature variation. On the other hand, magnesium-manganese series ferrites have defects such as low Curie temperatures and the concomitant unfavorable temperature stability of the saturation magnetization. Therefore, the object of the present invention is to eliminate these defects and to provide microwave circuit element materials for use in the VHF, UHF or SHF band range, having excellent characteristics such as low  $4\pi Ms$  values of less than 800 gauss, low ferromagnetic resonance linewidth values, and high Curie temperatures.

The garnet compositions are generally expressed by a normal formula unit  $\{A_3\}[B_2](C_3)O_{12}$ , wherein brackets  $\{ \}$ ,  $[ ]$  and  $( )$  represent respectively the 24c, 16a and 24d sites and A, B and C denote atoms occupying the respective sites. Fe has a preference for the two different sublattice sites (the 16a and the 24d sites) and the Fe-Fe superinteractions in each of and between these sublattice sites cause the Fe magnetic moments at the 16a and 24d sites to be coupled antiferromagnetically. Under the situation of the relative site unbalance, wherein the magnetic moment at the 24d site is not equal to that at the 16a site, the garnet compositions manifest ferrimagnetism. It has been generally considered that the compositions manifest antiferromagnetism in case of the site balance and at which an abnormal phenomenon of  $\Delta H$  occurs.

The value of  $4\pi Ms$  is determined by the relative site unbalance in the magnetic moment between the 16a and 24d sites for which Fe has a strong preference, while the temperature variation of  $4\pi Ms$  changes with the numbers of iron ions located on each sublattice site, kinds of nonmagnetic ions replacing the iron ions, and kinds of ions located on the 24c site.

The conventional calcium-vanadium garnet which can be expressed by a normal formula unit  $\{Ca_3\}[Fe_2](Fe_{1.5}V_{1.5})O_{12}$  was of little or no utility in that its  $\Delta H$  values were in excess of 300 oersteds in spite of its advantage of possessing a high Curie temperature and low  $4\pi Ms$  values. It has been found possible in accordance with the instant invention to lower the values of  $\Delta H$  by various substitutions in the calcium-vanadium garnet composition while preserving its above-mentioned advantages and also to prepare magnetic materials having characteristics superior to the conventional Ca-V garnet material.

According to this invention, excellent magnetic materials for use in VHF, UHF or SHF band range, featuring sufficiently low  $\Delta H$  values, high Curie temperatures,  $4\pi Ms$  values controllable within suitable ranges, small temperature variations in the value of  $4\pi Ms$  low manufacturing costs are obtained by the substitution of ions located on the 24c and 24d sites in Ca-V garnets with yttrium (Y) and germanium (Ge) ions and by the further substitution of ions on the 16a site with tantalum (Ta) ions.

The Ca-V garnet compositions substituted with Y and Ge of this invention are expressed by the chemical formula:



in which the values of x and y are required to lie within the polygonal area bounded by the lines connecting the coordinates:

|    | x    | y    |
|----|------|------|
| 20 | 0.05 | 0.05 |
|    | 0.8  | 0.05 |
|    | 1.8  | 1.1  |
|    | 0.5  | 2.4  |
|    | 0.05 | 2.4  |

on the x-y rectangular coordinates plane. Where the difference between the numbers of Fe ions located on the 16a site and the 24d site is 0.025 or less, an abnormal phenomenon of  $\Delta H$  is observed and the values of  $\Delta H$  cannot be improved. Of course, ferrimagnetism disappears if the difference is zero. Thus, the range of  $|2-(1.5-0.5x+0.5y)| \leq 0.025$ , i.e.,  $0.95 \leq y-x \leq 1.05$ , should be excluded from the above-mentioned effective range for x and y of the Y-and Ge-substituted Ca-V garnet compositions of this invention.

According to this invention, the Y-and Ge-substituted Ca-V garnets can be further substituted with Ta. The garnet compositions thus obtained can be expressed as

$\{Ca_{3-y}Y_y\}[Fe_{2-z}Ta_z](Fe_{1.5-0.5x+0.5y-z}Ge_xV_{1.5-0.5x-0.5y-z})O_{12}$ , in which x, y and z should be within the ranges  $0.05 \leq x \leq 0.8$ ,  $0.05 \leq y \leq 1.4$  and  $0 < z \leq 0.17$ , and preferably the ranges  $0.1 \leq x \leq 0.8$ ,  $0.05 \leq y \leq 1.4$  and  $0.02 \leq z \leq 0.17$ , respectively. Where the difference of the numbers of Fe ions between 16a and 24d sites  $|(2-z)-(1.5-0.5x+0.5y+z)|$  is 0.025 or less, the abnormal phenomenon of  $\Delta H$  is observed, as mentioned previously. Accordingly, the compositions satisfying the relation  $0.95 \leq 4z+y-x \leq 1.05$  should be excluded.

Furthermore, it is preferable to exclude a wider range of compositions in which the difference is 0.1 or less, that is  $0.8 \leq 4z+y-x \leq 1.2$ , in view of the effect on the improvement of  $\Delta H$ .

Both of the garnet compositions of this invention may be produced by presintering a mixture of oxides of the elements to be contained in the final product or a mixture of other compounds of such elements, which are easily decomposed into the respective oxides at elevated temperature, at a temperature or temperatures within the range of 800° to 1,150° C. for 1 to 8 hours in an oxidizing atmosphere, crushing and press-molding it, followed by sintering the molded body at a temperature or temperatures within the range of 1,160° to 1,350° C. for 1 to 30 hours in an oxidizing atmosphere.

Now a more detailed description and examples of this invention will be described by reference to the accompanying drawings, in which

FIG. 1 is a graph of the  $4\pi Ms$  versus temperature characteristics of the garnet compositions of the prior art and of this invention which illustrates the advantages of this invention;

FIGS. 2 and 3 show, respectively, ferromagnetic resonance linewidths ( $\Delta H$ ) and Curie temperatures as a function of x for the Y-and Ge-Substituted Ca-V ferrimagnetic garnets of this invention with the compositions expressed as



FIGS. 4, 5 and 6 show, respectively, Curie temperatures, ferromagnetic resonance linewidths ( $\Delta H$ ) and saturation magnetizations ( $4\pi Ms$ ) as a function of y for the same compositions as in FIGS. 2 and 3;

FIG. 7 is a composition diagram illustrating the effective range bounded by the lines connecting the coordinates ex-

pressed by  $(x,y)$  within which the Y- and Ge-Substituted Ca-V series ferrimagnetic garnet compositions according to this invention fall and the points of the coordinates  $(x,y)$  for typical garnet compositions listed in table 2;

FIGS. 8 and 9 are graphs respectively illustrating the influence of  $z$  (Ta) on  $\Delta H$  and  $4\pi Ms$  for the compositions expressed as



FIGS. 10 and 11 are graphs illustrating the influence of  $x$  (Ge) on  $\Delta H$  and  $4\pi Ms$  for the same compositions where  $y=0.4$  and  $z=0.1$ , respectively; and

FIGS. 12 and 13 are graphs illustrating the influence of  $y$  (Y) on  $\Delta H$  and  $4\pi Ms$  for the same compositions where  $x=0.4$ ,  $z=0.1$  and  $x=0.6$ ,  $z=0.1$ , respectively.

Referring first to FIG. 1 and table 1, the effects of the Ge- and Y-Substitutions and Ge-, Y-, and Ta-substitutions on the Ca-V garnets will be outlined.

Starting materials  $CaCO_3$ ,  $Fe_2O_3$ ,  $V_2O_5$ ,  $Ta_2O_5$ ,  $GeO_2$ , and  $Y_2O_3$  in such amounts were weighed, 350 grams in total in each case, so that each of the compositions shown in table 1 may be finally obtained. These materials were admixed in a ball mill made of steel, presintered at  $900^\circ C$ . for 4 hours, compressed into the desired shapes, and then sintered at  $1210^\circ C$ . for 20 hours in air. The sintered products were removed from the furnace when the furnace temperature cooled down to  $300^\circ C$ . Then the values of the saturation magnetization ( $4\pi Ms$ ) at room temperature ( $23^\circ-25^\circ C$ ), the linewidth ( $\Delta H$ ) at 9 GHz., and the Curie temperature were measured.

Table 1 lists the results of measurements for the unsubstituted, tantalum-substituted, tantalum-and germanium-substituted, yttrium and germanium-substituted and tantalum-, germanium-, and yttrium-substituted Ca-V series garnet compositions to demonstrate the successively promoted substitution effects, as regards a decrease in the linewidth  $\Delta H$  and an increase in the Curie temperature.

TABLE I

| Composition                                                                                                                                                 | $4\pi Ms$<br>(gauss) | $\Delta H$<br>(oersteds) | Curie<br>tem-<br>pera-<br>ture<br>( $^\circ C$ ) |
|-------------------------------------------------------------------------------------------------------------------------------------------------------------|----------------------|--------------------------|--------------------------------------------------|
| Sample No:                                                                                                                                                  |                      |                          |                                                  |
| I-----<br>[Ca <sub>3</sub> ][Fe <sub>2</sub> ](Fe <sub>1.5</sub> V <sub>1.5</sub> )O <sub>12</sub>                                                          | 520                  | 370                      | 220                                              |
| II-----<br>[Ca <sub>3</sub> ][Fe <sub>1.9</sub> Ta <sub>0.1</sub> ](Fe <sub>1.6</sub> V <sub>1.4</sub> )O <sub>12</sub>                                     | 310                  | 170                      | 205                                              |
| III-----<br>[Ca <sub>3</sub> ][Fe <sub>1.9</sub> Ta <sub>0.1</sub> ](Fe <sub>1.4</sub> Ge <sub>0.4</sub> V <sub>1.2</sub> )O <sub>12</sub>                  | 580                  | 85                       | 169                                              |
| IV-----<br>[Ca <sub>2.6</sub> Y <sub>0.4</sub> ][Fe <sub>2</sub> ](Fe <sub>1.6</sub> Ge <sub>0.4</sub> V <sub>1.0</sub> )O <sub>12</sub>                    | 580                  | 148                      | 218                                              |
| V-----<br>[Ca <sub>2.6</sub> Y <sub>0.4</sub> ][Fe <sub>1.9</sub> Ta <sub>0.1</sub> ](Fe <sub>1.6</sub> Ge <sub>0.4</sub> V <sub>1.0</sub> )O <sub>12</sub> | 365                  | 76                       | 209                                              |

Measured  $4\pi Ms$  values as a function of the temperature of the samples Nos. I through V contained in table 1 and also of aluminum-substituted YIG are illustrated in FIG. 1.

Sample No. I, or the unsubstituted Ca-V garnet composition, has no practical utilization in that its linewidth  $\Delta H$  is as high as 370 with a resulting large magnetic loss, although it possesses a low  $4\pi Ms$  value and a high Curie temperature.

The effectiveness of tantalum-substitution in the sample No. II composition can be understood from a decrease in  $4\pi Ms$  caused by the substitution of Fe ion on the  $16a$  site with Ta and at the same time, a decrease in  $\Delta H$ , to a value of  $\Delta H=170$ , less than one-half of that of the unsubstituted Ca-V garnet. A further decrease in the value of  $\Delta H$ , to a value of  $\Delta H=85$ , is achieved by a further substitution of Fe ion on the  $24d$  site with Ge as indicated in the sample No. III composition. This value is less than one-fourth of the value of  $\Delta H$  of sample No. I composition and is one-half of the value of  $\Delta H$  of sample No. II composition. A defect of the Ta- and Ge-substitution, however, is a remarkable decrease in the Curie temperature, which in turn causes an increase in the temperature variation of  $4\pi Ms$ .

This defect can be improved by substituting some fraction of Ca-ions on the  $24c$  site with Y-ions instead of by Ta-substitution as shown in sample No. IV. This composition has a higher Curie temperature. Though  $\Delta H$  is increased in comparison with sample No. III, it is possible to have a lower  $\Delta H$  value with a sufficiently high Curie temperature by changing

the amounts of substitution and other parameters. The defect of sample No. III can be also improved by further substituting Ca-ions with Y-ions in addition to the Ge- and Ta-substitutions as shown in the sample No. V composition. This garnet composition possesses a lower  $4\pi Ms$  and a lower  $\Delta H$  value ( $\Delta H = 76$  the Y-, Ge- and Ta-substitutions have succeeded in raising the Curie temperature which was lowered by the Ge- and Ta-substitutions in the composition of sample No. III. Thus it has become possible to provide a composition having both a high Curie temperature and an excellent  $4\pi Ms$  versus temperature characteristics as indicated in FIG. 1. In such a manner, magnetic materials can be prepared, which possess low  $4\pi Ms$ , low  $\Delta H$ , high Curie temperatures, and improved  $4\pi Ms$  versus temperature characteristics, by substituting Ca-V garnets with Y and Ge or with Ta, Y and Ge.

Now examples and the effective range of the Y- and Ge-substituted Ca-V garnet compositions will be described with reference to FIGS. 2 through 7.

In preparing the samples, starting materials  $CaCO_3$ ,  $Fe_2O_3$ ,  $V_2O_5$ ,  $GeO_2$ , and  $Y_2O_3$  each in varying amounts in the compositions:

$\{Ca_{3-y}Y_y\}[Fe_2](Fe_{1.5-0.5x+0.5y}Ge_xV_{1.5-0.5x-0.5y})O_{12}$

were weighed, admixed in a ball mill made of steel, presintered at  $900^\circ C$ . for 4 hours, compressed into desired shapes, followed by a sintering process at  $1,260^\circ C$ . in air for 15 hours. The sintered bodies were removed from the furnace when the furnace temperature cooled down to  $300^\circ C$ . Then measurements of saturation magnetization ( $4\pi Ms$ ) at room temperature ( $23^\circ-25^\circ C$ ), linewidth ( $\Delta H$ ) at 9.5 GHz. and Curie temperature were conducted.

Referring to FIG. 2 illustrating the measurement result, it will be seen that linewidth ( $\Delta H$ ) decreases with increasing  $x$  for  $y=0$  as indicated by curve a. Curve b is for  $y=0.5$  and a decrease in  $\Delta H$  also occurs with increasing  $x$ . Curve c is for  $y=1.1$ , in which  $\Delta H$  reaches the compensation point at  $x=0.1$ .

and at this point it manifests an abnormal phenomenon. But even as for curves a and b,  $\Delta H$  decreases with increasing  $x$ . As is clearly seen, an increase in  $x$ —that is, large substitutions of  $GeO_2$ , is very effective in lowering the values of the linewidth ( $\Delta H$ ).

As shown in FIG. 3, however, an increase in  $x$  causes a decrease in the Curie temperature. Curves a, b, and c show respectively Curie temperatures as a function of  $x$  for  $y=0$ ,  $y=0.5$ , and  $y=1.1$ . A rapid decrease in the Curie temperature can be observed in the curve a—that is, the Curie temperature of  $107^\circ C$ . at  $x=0.8$  drops to lower than  $100^\circ C$ . for an  $x$  value in excess of 0.8. The materials having  $y=0$  and  $x$  exceeding 0.8 are of little utility in that the temperature stability of  $4\pi Ms$  is exceedingly low. When the substitution quantity of  $Y_2O_3$ , or the value of  $y$ , is increased under these circumstances, the Curie temperature becomes lower than  $100^\circ C$ . only after the point  $x=1.2$  has been exceeded in the case of curve b or  $y=0.5$ , while in case of curve c, or  $y=1.1$ , the Curie temperature remains higher than  $100^\circ C$ . down to the point  $x=1.8$ . In such a way, increasing the value of  $y$  causes higher Curie temperatures and a more gradual decrease in the slope of the plot of Curie temperature versus  $x$ . Stated more particularly, the decrease in the Curie temperature due to an increase in  $x$  from 0 to 1.0 in curves a ( $y=0$ ), b ( $y=0.5$ ), and c ( $y=1.1$ ) is respectively  $130^\circ$ ,  $118^\circ$ , and  $88^\circ$  centigrade. This indicates clearly that the rate of decrease of the Curie temperature becomes smaller with increasing  $y$ .

To demonstrate the effect of this invention for raising the Curie temperature with increasing  $y$ , the dependence of Curie temperature on  $y$  in the case of  $x=0.5$  is shown in FIG. 4. As is evident from the figure, the Curie temperature becomes higher with increasing  $y$ . In other words, the temperature variation of the value of  $4\pi Ms$  with an increase in  $y$  has been outstandingly improved.

Our experiment has demonstrated that an increase in  $y$  causes higher Curie temperatures irrespective of the values of  $x$ .

Marked improvements in the value of the linewidth ( $\Delta H$ ) with increasing  $y$ —that is, with larger  $Y_2O_3$  substitutions, can be also observed, as shown in FIG. 5.

Referring to FIG. 5, curve  $a$  indicates the linewidth  $\Delta H$  as a function of  $y$  for  $x=0.5$ . At first,  $\Delta H$  decreases with an increase in  $y$  and reaches a minimum  $\Delta H=180$  at  $y=0.5$ . With a further increase in the value of  $y$ ,  $\Delta H$  begins to increase and reaches the compensation point at  $y=1.05$ , at which an abnormal phenomenon of  $\Delta H$  can be observed. With a still further increase in  $y$ ,  $\Delta H$  decreases until it reaches a minimum at about  $y=1.8$  and thereafter, increases again. In case  $y$  exceeds 2.4, the linewidth  $\Delta H$  becomes degraded as compared with that for  $y=0$  or that of the composition not substituted with  $Y_2O_3$ .

Curve  $b$  indicates  $\Delta H$  as a function of  $y$  for  $x=0.5$ . At first, a decrease in  $\Delta H$  occurs with increasing  $y$ ,  $\Delta H$  reaching an excellent value  $\Delta H=53$  at  $y=0.4$ . Thereafter  $\Delta H$  begins to increase with an increase in  $y$  to reach the saturation point at  $y=1.5$ , at which point an abnormal phenomenon of  $\Delta H$  can be observed. Thereafter  $\Delta H$  begins to decrease again with increasing  $y$ , reaching a minimum  $\Delta H=200$  at  $y=2.0$ . Beyond the point  $y=2.4$ , the value of  $\Delta H$  becomes larger than that of the composition not substituted with  $Y_2O_3$  for  $x=0.05$ , which is 290.

As will be evident from the foregoing description, an increase in  $y$  causes marked improvements not only in Curie temperature, but also in linewidth ( $\Delta H$ ).

FIG. 6 shows the dependence of  $4\pi Ms$  on  $y$  for  $x=0.5$ . The value of  $4\pi Ms$  decreases at first with increasing  $y$  and the composition at  $y=1.5$  manifests the antiferromagnetic properties. Thereafter  $4\pi Ms$  increases with increasing  $y$ . As is evident,  $4\pi Ms$  can take any desired values less than 800 gauss with varying values of  $y$ . This is advantageous in employing the present materials in the VHF, UHF or SHF band range.

Conventional materials with low  $4\pi Ms$  values have been considered to be of little utility because of their low Curie temperatures, unfavorable temperature stability of  $4\pi Ms$  and high magnetic losses. Therefore, the Ca-V series garnets having low  $4\pi Ms$ , low linewidths, and high Curie temperatures prepared in accordance with this invention are unprecedented heretofore. For instance, the indicated Ca-V garnet materials possess the excellent performance such as  $4\pi Ms=260$ ,  $\Delta H=96$ , Curie temperature =  $228^\circ C.$ , for  $x=0.5$  and  $y=1.0$ . The yttrium-iron-aluminum series garnets and magnesium-manganese series ferrites currently used as microwave device materials have been found inadequate for the following reasons: The Curie temperature approaches  $100^\circ C.$ , for  $4\pi Ms$  values of the order of 260 gauss, which causes an increase in the temperature variation of  $4\pi Ms$  and a drift of tuning points due to temperature variations. This results in a degradation in the isolation property, an increase in the VSWR, and an increase in the insertion loss.

As will be apparent, this invention can provide calcium-vanadium series ferrimagnetic garnets with high Curie temperatures, low  $\Delta H$ , low  $4\pi Ms$  values, and a small temperature variation of  $4\pi Ms$ , which are suitable for use in microwave devices operating, notably, in the VHF, UHF and SHF band range.

Table 2 contains a listing of many exemplary samples of the Ca-V ferrimagnetic garnets having varying values of  $x$  and  $y$  and obtained at various sintering conditions (sintering temperature and time intervals) to clarify the advantages of this invention.

TABLE 2

| 5           | x    | y    | Sintering conditions |      | $4\pi Ms$<br>(gauss) | $\Delta H$<br>(oersteds) | Curie<br>tem-<br>pera-<br>ture<br>( $^\circ C.$ ) |
|-------------|------|------|----------------------|------|----------------------|--------------------------|---------------------------------------------------|
|             |      |      | $^\circ C.$          | Hrs. |                      |                          |                                                   |
| Sample No.: |      |      |                      |      |                      |                          |                                                   |
| 1           | 0.8  | 0    | 1,210                | 10   | 78                   | 80                       | 97                                                |
| 2           | 0.5  | 0.05 | 1,230                | 20   | 715                  | 118                      | 153                                               |
| 3           | 0.5  | 0.2  | 1,210                | 20   | 760                  | 75                       | 176                                               |
| 4           | 0    | 0.5  | 1,210                | 20   | 290                  | 180                      | 260                                               |
| 5           | 0.05 | 0.5  | 1,210                | 20   | 320                  | 169                      | 255                                               |
| 6           | 0.5  | 0.5  | 1,210                | 20   | 503                  | 83                       | 197                                               |
| 7           | 0.5  | 0.5  | 1,250                | 20   | 513                  | 51                       | 200                                               |
| 8           | 1.2  | 0.5  | 1,230                | 20   | 503                  | 41                       | 145                                               |
| 9           | 1.0  | 1.0  | 1,300                | 8    | 123                  | 49                       | 103                                               |
| 10          | 1.6  | 1.2  | 1,300                | 20   | 680                  | 130                      | 143                                               |
| 11          | 0    | 1.5  | 1,300                | 15   | 360                  | 248                      | 274                                               |
| 12          | 0.3  | 1.5  | 1,300                | 15   | 98                   | 221                      | 269                                               |
| 13          | 1.0  | 1.5  | 1,300                | 15   | 315                  | 120                      | 182                                               |
| 14          | 1.4  | 1.5  | 1,300                | 5    | 300                  | 94                       | 178                                               |
| 15          | 0.6  | 2.0  | 1,300                | 20   | 325                  | 140                      | 259                                               |
| 16          | 0.7  | 2.2  | 1,300                | 20   | 400                  | 136                      | 251                                               |
| 17          | 0.2  | 2.4  | 1,300                | 5    | 783                  | 181                      | 277                                               |
| 18          | 0.2  | 2.4  | 1,350                | 5    | 790                  | 122                      | 277                                               |
| 19          | 0.05 | 0.05 | 1,210                | 20   | 140                  | 49                       | 109                                               |
| 20          | 1.8  | 1.1  | 1,250                | 20   | 80                   | 50                       | 100                                               |
| 21          | 0.5  | 2.4  | 1,300                | 15   | 420                  | 270                      | 272                                               |
| 22          | 0.05 | 2.4  | 1,300                | 15   | 435                  | 281                      | 280                                               |
| 23          | 1.9  | 1.1  | 1,250                | 20   | 49                   | 50                       | 72                                                |
| 24          | 0    | 0    | 1,210                | 10   | 620                  | 290                      | 225                                               |
| 25          | 0.6  | 2.4  | 1,300                | 20   | 450                  | 320                      | 258                                               |
| 26          | 0    | 2.4  | 1,300                | 20   | 520                  | 290                      | 280                                               |
| 27          | 0.3  | 1.0  | 1,300                | 5    | 180                  | 178                      | 240                                               |
| 28          | 0.1  | 2.0  | 1,300                | 15   | 520                  | 229                      | 277                                               |
| 29          | 0.2  | 0.2  | 1,210                | 20   | 588                  | 126                      | 212                                               |

Note.—Sample numbers bearing an asterisk (\*) denote compositions not included in the scope of the instant invention.

The effectiveness of the present invention in causing a marked improvements in linewidth will be readily evident from an examination of  $\Delta H$  values for various compositions as shown in table 2.

Thus, varying the values of  $x$  and  $y$ —that is, varying the amounts of  $Ge_2O_3$  and  $Y_2O_3$  substitutions, in the calcium-vanadium series garnet compositions which can be expressed as

$\{Ca_{3-y}Y_y\}[Fe_2](Fe_{1.5-0.5x+0.5y}Ge_xV_{1.5-0.5x-0.5y})O_{12}$  enables high Curie temperatures and low linewidth ( $\Delta H$ ) values which are much lower than the values of  $\Delta H$  of the unsubstituted calcium vanadium garnet compositions.

The  $x$  and  $y$  values in the compositions of this invention lie, as mentioned previously, within the polygonal area A-B-C-D-E shown in FIG. 7 which is bounded by the lines connecting the coordinates:

| 50 | x    | y    |
|----|------|------|
| A  | 0.05 | 0.05 |
| B  | 0.8  | 0.05 |
| C  | 1.8  | 1.1  |
| D  | 0.5  | 2.4  |
| E  | 0.05 | 2.4  |

From the area A-B-C-D-E, the range of  $0.95 \leq y-x \leq 1.05$  should be excluded, as mentioned previously.

The reason why the area A-B-C-D-E is defined is as follows:

The compositions outside the lines A-B and E-A manifest to an insufficient degree the beneficial effects of this invention to render them useful in practical applications; the compositions lying in the area above the line B-C possess low Curie temperatures less than  $100^\circ C.$  and large temperature variations of  $4\pi Ms$ , rendering them difficult for practical use, although they have improved  $\Delta H$  values; the compositions lying outside of the line C-D and having relatively small values of  $y$  possess low Curie temperatures and large temperature variations of  $4\pi Ms$ ; in the compositions outside the line C-D and having a larger value for  $y$ ,  $\Delta H$  values are not substantially improved; the compositions lying outside of the line D-E have high Curie temperatures, but their  $\Delta H$  values are substantially the same as or a little inferior to the  $\Delta H$  value of the unsubstituted Ca-V garnet compositions. In order to improve the  $\Delta H$  values of compositions with  $y$  values larger than those of the compositions of the instant invention, sintering for long

time intervals at extremely elevated temperatures would be necessary, which apparently does not meet the objects of this invention.

Now the effect of Ta-substitution combined with Ge- and Y-substitutions will be clarified with reference to FIGS. 8 to 13.

Samples hereinafter referred to which are expressed as



and have the values of  $x=0 \approx 1.0$ ,  $y=0 \approx 1.6$ , and  $z=0 \approx 0.4$  were produced and measured in the same manner as used for the compositions of table 1. Referring to FIG. 8 illustrating the dependence of  $z(Ta)$  on  $\Delta H$  where  $x=0.4$  and  $y=0.4$ , the value of  $\Delta H$  which is 148 at  $z=0$  gradually decreases with increasing  $z$ , reaching a minimum  $\Delta H=76$  at  $z=0.1$ . Further substitution of Ta causes  $\Delta H$  to increase. In excess of  $z=0.17$ , the value of  $\Delta H$  becomes equal to that at  $z=0$ . Further increase in  $z(Ta)$  causes an increase in  $\Delta H$ , or deterioration of  $\Delta H$ , beyond the initial value until the point  $z=0.25$  has been reached at which the 16a and 24d site unbalance in the number of Fe-ions disappears and ferrimagnetism is lost. As a result, the value of  $\Delta H$  becomes extremely high. As the value of  $z$  increases, such as to 0.3 or 0.4, the value of  $\Delta H$  decreases accordingly.

FIG. 9 indicates the influence of  $z(Ta)$  on the value of  $4\pi Ms$  where  $x$  and  $y$  are both 0.4. An increase in the amount of substitution of Ta causes a decrease in  $4\pi Ms$  and the value of  $4\pi Ms$  becomes extremely low at  $z=0.25$  at which the 16a and 24d site unbalance disappears. The increased substitution, such as to values of  $z=0.3$  or 0.4, causes an increase in  $4\pi Ms$  again.

The manner in which the Curie temperature decreases with an increase in  $z(Ta)$  is shown in table 3.

TABLE 3

| x   | y   | z    | Curie temp. (°C.) |
|-----|-----|------|-------------------|
| 0.4 | 0.4 | 0    | 218               |
| 0.4 | 0.4 | 0.1  | 209               |
| 0.4 | 0.4 | 0.15 | 205               |
| 0.4 | 0.4 | 0.17 | 202               |
| 0.4 | 0.4 | 0.20 | 196               |
| 0.4 | 0.4 | 0.30 | 181               |
| 0.4 | 0.4 | 0.40 | 166               |

As heretofore mentioned, substitution by Ta causes a decrease in  $4\pi Ms$  in spite of its small amounts. Notably in the range  $z=0 \approx 0.17$ , the substitution is also effective for lowering the value of  $\Delta H$ . As  $z=0.17$  is exceeded, however,  $\Delta H$  becomes higher than its initial value at  $z=0$ , while for large values of  $z$  the Curie temperature becomes low. Therefore, the effective  $z$  range is the  $0 < z \leq 0.17$ . Since substitution effect is limited for values of  $z$  less than 0.02, the preferable  $z$  range is  $0.02 \leq z \leq 0.17$ .

FIG. 10 indicates the influence of  $x$  (Ge) on  $\Delta H$  in the composition where  $y=0.4$  and  $z=0.1$ . The value of  $\Delta H$ , which is 220 at  $x=0$ , decreases with an increase in  $x$  and reaches 25 at  $x=0.8$ .

FIG. 11 shows the dependence of  $4\pi Ms$  on  $x$  in the same case. The value of  $4\pi Ms$  increases with increasing  $x$ , becoming more than 600 gauss at  $x=0.8$ .

Changes in Curie temperature in this case are listed in table 4. It will be seen that the Curie temperature decreases with increasing  $x$  and becomes lower than 150° C. for values of  $x$  in excess of  $x=0.8$ , resulting in an increase in the temperature variation of  $4\pi Ms$ . Therefore, the effective  $x$  values are in the range  $0.05 \leq x \leq 0.8$ . Since substitution effect is limited for values of  $x=0.1$  as is apparent from FIG. 10, the range of  $x$  values is preferably  $0.1 \leq x \leq 0.8$ .

TABLE 4

| x   | y   | z   | Curie temp. (°C.) |
|-----|-----|-----|-------------------|
| 0   | 0.4 | 0.1 | 230               |
| 0.2 | 0.4 | 0.1 | 218               |
| 0.4 | 0.4 | 0.1 | 209               |
| 0.6 | 0.4 | 0.1 | 192               |
| 0.8 | 0.4 | 0.1 | 152               |
| 1.0 | 0.4 | 0.1 | 101               |

FIG. 12 indicates the influence of  $y$  (Y) on  $\Delta H$  in the cases of  $x=0.4$  and  $z=0.1$  (curve a) and  $x=0.6$  and  $z=0.1$  (curve b). The value of  $\Delta H$  at  $y=0$  for the curve a is 139 and an increase in  $y$  causes a decrease in  $\Delta H$ , the value reaching 50 at  $y=0.2$ . Then, the value of  $\Delta H$  increases with an increase in  $y$  and, at  $y=1.0$ , the relative 16a and 24d site unbalance in the Fe-ion number disappears and an abnormal phenomenon of  $\Delta H$  occurs. Thenceforth a decrease in  $\Delta H$  occurs again with an increase in  $y$ , reaching  $\Delta H=110$  at  $y=1.4$ . At  $y=1.6$ , the value of  $\Delta H$  begins to increase. This is because the sintering temperature becomes higher according as the quantity of yttrium substitution is increased.

In case of curve b, the value of  $\Delta H$ , which is 75 at  $y=0$ , begins to decrease with an increase in  $y$ , reaching 39 at  $y=0.2$ . Thereafter the value of  $\Delta H$  begins to increase with increasing  $y$ . At  $y=1.2$ , the 16a and 24d site unbalance disappears, at which point the value of  $\Delta H$  becomes exceedingly high. Thenceforth the value of  $\Delta H$  decreases gradually with an increase in  $y$ .

FIG. 13 illustrates the dependence of  $4\pi Ms$  on the value of  $y$  in the same case. With an increase in  $y$ , i.e., yttrium substitution quantities, the value of  $4\pi Ms$  decreases. In case of  $x=0.4$  and  $z=0.1$  (curve a), the 16a and 24d site unbalance occurs at  $y=1.0$ , while in case of  $x=0.6$  and  $z=0.1$  (curve b), at  $y=1.2$ . Under this situation, the  $4\pi Ms$  value becomes less than 50. This point corresponds to approximately the point where the relation  $4z+y-x=1$  is satisfied. It is generally considered that compositions meeting this relationship manifest antiferromagnetism and do not manifest ferrimagnetism.

The Curie temperatures increase with an increase in  $y$  as shown in table 5 and this increase tends to compensate for a decrease in Curie temperature caused by the combined tantalum- and germanium-substitutions. An increase in  $y$  causes higher Curie temperatures as is evidenced by the fact that a value of 180° C. in case of  $x=0.4$ ,  $z=0.1$  and  $y=0$  increases to 258° C. in case of  $x=0.4$ ,  $z=0.1$ , and  $y=1.4$ , and the improved  $4\pi Ms$  versus temperature characteristic. But an increase in  $y$  is disadvantageous in the use of large quantities of  $Y_2O_3$  which is an expensive raw material. This inevitably renders finished material costs expensive. Furthermore, large yttrium substitutions call for higher sintering temperatures, which are not suited to large-scale industrial production. On the other hand, values of  $y$  less than 0.05 manifest little of the yttrium substitution effect of yttrium. Therefore the effective range of  $y$  is determined as  $0.05 \leq y \leq 1.4$ .

TABLE 5

| x   | y   | z   | Curie temp. (°C.) |
|-----|-----|-----|-------------------|
| 0.4 | 0   | 0.1 | 180               |
| 0.4 | 0.1 | 0.1 | 191               |
| 0.4 | 0.2 | 0.1 | 198               |
| 0.4 | 0.4 | 0.1 | 209               |
| 0.4 | 0.6 | 0.1 | 222               |
| 0.4 | 0.8 | 0.1 | 232               |
| 0.4 | 1.4 | 0.1 | 258               |
| 0.6 | 0.2 | 0.1 | 182               |
| 0.6 | 0.4 | 0.1 | 195               |
| 0.6 | 0.8 | 0.1 | 213               |
| 0.6 | 1.4 | 0.1 | 246               |

Thus, with the tantalum-, germanium- and yttrium-sub-

stituted calcium-vanadium series garnet materials, excellent  $\Delta H$  values, low  $4\pi Ms$ , high Curie temperatures and a low cost can be realized. Also, better  $4\pi Ms$  versus temperature characteristics than the aluminum-substituted YIG is obtained as are evident from FIG. 1. For instance, the Curie temperature of the aluminum-substituted YIG indicated by YIG (A1) in the figure which have a  $4\pi Ms$  value of about 350 gauss at room temperature is at or near 120° C., and hence the temperature variation of  $4\pi Ms$  is quite large. One of the compositions of this invention which is indicated by curve No. V in FIG. 1 possesses a  $4\pi Ms$  value at room temperature of 365 gauss and Curie temperature of 209° C. at which  $4\pi Ms$  becomes 0. The  $4\pi Ms$  versus temperature characteristics of this composition are quite superior to those of the aluminum-substituted YIG.

As has been mentioned, the Ca-V series ferromagnetic garnets according to this invention offer advantages over the known yttrium-iron-aluminum garnets series of low- $4\pi Ms$  microwave magnetic materials such as lower magnetic losses, higher Curie temperatures, improved  $4\pi Ms$  versus temperature characteristics, lower costs which comes from the use of smaller quantities of yttrium, and also lower sintering temperatures (of the order of as low as 200° C.) than those of the aluminum-substituted YIG, which advantages can be important in large-scale industrial production.

The compositions of the invention provide inexpensive microwave element materials for use in VHF, UHF and SHF band ranges, the materials having low  $4\pi Ms$  values, improved  $4\pi Ms$  versus temperature characteristics, low magnetic losses and being also easily amenable to large-scale production. The tantalum-germanium-yttrium substituted calcium-vanadium garnet compositions are particularly useful in this regard as follows:

{Ca<sub>3-y</sub>Y<sub>y</sub>} [Fe<sub>2-z</sub>Ta<sub>z</sub>] (Fe<sub>1.5-0.5x+0.5y+z</sub>Ge<sub>x</sub>V<sub>1.5-0.5x-0.5y-z</sub>)<sub>12</sub>  
wherein the ranges 0.05 ≤ x ≤ 0.8, 0.05 ≤ y ≤ 1.4, and 0 < z ≤

35

40

45

50

55

60

65

70

75

0.17, and preferably 0.1 ≤ x ≤ 0.8, 0.05 ≤ y ≤ 1.4 and 0.02 ≤ z ≤ 0.17 are employed, from which the values of x, y, and z determined by the relation 0.95 ≤ 4z+y-x ≤ 1.05 and preferably 0.8 ≤ 4z+y-x ≤ 1.2 are excluded.

What is claimed is:

1. Calcium-vanadium ferrimagnetic garnets having the compositions expressed by the formula:

{Ca<sub>3-y</sub>Y<sub>y</sub>} [Fe<sub>2-z</sub>Ta<sub>z</sub>] (Fe<sub>1.5-0.5x+0.5y+z</sub>Ge<sub>x</sub>V<sub>1.5-0.5x-0.5y-z</sub>)<sub>12</sub>  
wherein values of x and y lie within the polygonal area A-B-C-D-E shown in FIG. 7 of the drawing which is bounded by the lines connecting the coordinates:

|   | x    | y    |
|---|------|------|
| A | 0.05 | 0.05 |
| B | 0.8  | 0.5  |
| C | 1.8  | 1.1  |
| D | 0.5  | 2.4  |
| E | 0.05 | 2.4  |

and wherein the range expressed by the relation 0.95 ≤ y-x ≤ 1.05 is excluded from said area.

2. Calcium-vanadium ferrimagnetic garnets having compositions expressed by the formula:

{Ca<sub>3-y</sub>Y<sub>y</sub>} [Fe<sub>2-z</sub>Ta<sub>z</sub>] (Fe<sub>1.5-0.5x+0.5y+z</sub>Ge<sub>x</sub>V<sub>1.5-0.5x-0.5y-z</sub>)<sub>12</sub>  
wherein values of x, y and z are in the ranges expressed as 0.5 ≤ x ≤ 0.8; 0.05 ≤ y ≤ 1.4 and 0 < z ≤ 0.17, respectively, but excluding the values of x, y and z determined by the relation 0.95 ≤ 4z+y-x ≤ 1.05.

3. Calcium-vanadium series ferrimagnetic garnets as claimed in claim 2, wherein the values of x, y and z are in the ranges of 0.1 ≤ x ≤ 0.8; 0.05 ≤ y ≤ 1.4 and 0.02 ≤ z ≤ 1.7, respectively, but excluding the values of x, y and z determined by the relation 0.8 ≤ 4z+y-x ≤ 1.2.

\* \* \* \* \*